

Mar. 3, 1925

P. D. RICHARDS

1,528,632

FLOOR COVERING

Filed Oct. 11, 1922

*Fig. 1*



*Fig. 2*



Inventor—  
Perry D. Richards.  
by his Attorneys—  
*Thomas Thomas*

## UNITED STATES PATENT OFFICE.

PERRY D. RICHARDS, OF LANSDOWNE, PENNSYLVANIA, ASSIGNOR TO CONGOLEUM COMPANY, INC., OF NEW YORK, N. Y., A CORPORATION OF NEW YORK

## FLOOR COVERING.

Application filed October 11, 1922. Serial No. 593,809.

To all whom it may concern:

Be it known that I, PERRY D. RICHARDS, a citizen of the United States, residing in Lansdowne, Delaware County, Pennsylvania, have invented certain Improvements in Floor Coverings, of which the following is a specification.

One object of my invention is to provide a substantial felt base for a floor covering of the oil cloth or linoleum type.

A further object of the invention is to make a felt base having a large proportion of rags and hair bound by a bituminous binder.

In the accompanying drawings:

Fig. 1 is a perspective view of a small section of my improved felt base: and

Fig. 2 is a perspective view of the complete floor covering having my improved felt base.

In preparing the improved base, I use a percentage of rag fibres; a percentage of animal hair, preferably of considerable length, and a percentage of kraft sulphide pulp.

I have found that the following formula makes a substantial base: 50% rags (preferably cotton rags): 30% hair (domestic, and preferably long staple): 20% kraft sulphide pulp.

These ingredients are mixed thoroughly and felted into sheets in the ordinary manner. The sheets of felt are then impregnated with a bituminous compound, preferably an asphalt compound. This compound is heated to a proper degree. The felt to be saturated is passed through the hot bituminous liquid so that it is thoroughly impregnated, there being, however, no surplus of the binder. The saturation of the felt binds the cotton fibres and hair and a strong base is formed which will withstand a considerable amount of hard usage and which will not tear under severe torsional strains.

The felt base is then coated with a linseed oil, or a paint composition, on one face to prepare the face for the ornamental printed surface that is applied by the ordinary method of floor cloth printing. The back is preferably coated with a suitable paint composition to improve its appearance.

When my improved base is used as a backing for linoleum either in sheets or in sections, the method of applying the linoleum surface to the felt can be carried out in the usual manner.

When the felt base hereinbefore described is used as a body for printed hard surface floor covering, it adds materially to the quality of such floor covering over any that has been produced from the fact that it has all of the qualities of felt base material previously made, such as flexibility; ease of handling; laying flat on a floor without tacking, cementing or nailing; and, in addition, has the added strength, so that it will not tear easily, and may be cut to fit pipes, posts, or other projections in a room. It is non-absorbent, and, when made according to my claims, will not stain, or rub off on the floors, or surrounding carpets.

I claim:

1. As a new article of manufacture, a felt base for a floor covering of the oil cloth or linoleum type, consisting of finely divided rag fibres, animal hair and kraft sulphide pulp formed into a felted sheet and impregnated with a bituminous binder.

2. As a new article of manufacture, a felt base for floor covering of the oil cloth or linoleum type, consisting of substantially 50% finely divided cotton rags, 30% animal hair and 20% kraft sulphide pulp formed into felted sheets and impregnated with a bituminous binder.

PERRY D. RICHARDS.